

May 5, 1931.

H. S. MEARS

1,803,912

ROPE STRUCTURE

Filed Jan. 15, 1929



INVENTOR.

HENRY S. MEARS

BY

*H. S. Mears*  
ATTORNEY.

## UNITED STATES PATENT OFFICE

HENRY S. MEARS, OF PORTLAND, OREGON

## ROPE STRUCTURE

Application filed January 15, 1929. Serial No. 332,589.

My invention relates to an improvement in fiber rope, the invention being more specifically applicable to rope used for marine purposes.

5 Ropes intended for outdoor use, as for example marine ropes, should be made so as not to be affected by moisture to such extent as to become stiff and thus inflexible and hard to handle. This is a common fault in marine rope, due to the fact that in these ropes as ordinarily constructed the yarns are arranged in concentric circles with a relatively high number of turns per lineal unit to each yarn, so that the yarns do not lie closely together but rather across one another, thus forming interstices between them in which water collects and causes the fibers to become water-soaked and to swell and harden.

Furthermore, in ropes of this character, especially when wet, which is, of course, the normal condition of service of marine ropes, the yarns being more or less water-soaked and hence stiff and hard tend to resist individual relative adjustment to a bending stress 20 causing the rope to be very stiff, that is inflexible; and furthermore, since the yarns are hard and stiff they tend to cut and chafe causing the fibers of the rope to wear rapidly, and hence reducing its strength.

30 I have discovered that in order to prevent the fibers of a rope from becoming water-soaked and chafing and cutting, and thus setting up the said undesirable conditions it is necessary that the yarns composing the 35 strands be arranged so as to lie close together with practically no interstices between them, and further so as to constitute a substantially homogeneous mass, instead of merely a series of separate units each having to withstand 40 independently the strains imposed upon the rope.

To attain this arrangement the yarns composing the strands must be given a predetermined number of turns in one direction 45 per lineal unit, and the strands must be

given a relatively greater number of turns in the opposite direction for the same unit; whereby in the finished strand the yarns lying approximately on a circle concentric with the center of, and inscribed by the circumference of the strand, and enclosing approximately one-half the total area of the cross section of the core of the strand will have substantially no turns in either direction; the yarns lying on the interior of said circle will have turns in the same direction as the strand, but the amount of turn will be progressively increased toward the center; while the yarns located exterior of said circle will have turns opposite to those of the strand with the amount of such turns progressively increased towards the circumference of the strand.

These features and the details of construction of my improved rope are hereinafter 65 fully described with reference to the accompanying drawings.

In the drawings:

Fig. 1 shows diagrammatically a strand of my rope the yarns having received their 70 initial number of turns and assembled to form the strand, but before the strand has been twisted in the opposite directions;

Fig. 2 shows the strand of rope similarly to Fig. 1, except that the strand has received 75 its relatively greater number of turns in the opposite direction and illustrates by arrows the resultant relative turns of the yarns; and

Fig. 3 shows diagrammatically a section of rope embodying my invention.

Referring now to the figures, in Fig. 1 is shown the yarns *a* theoretically assembled to form a strand *b*, the strand being as yet un-twisted. The cover yarns *d* are cut away and may be disregarded as being no part of my invention. As will be noted the yarns *a* have been given an arbitrary initial number of turns to the left as represented by the arrow *A* and the strand *b* is to be twisted to the right as indicated by the arrow *B*.

In Fig. 2 the strand *b* has been given an arbitrary relatively greater number of turns to the right with the resulting effect on the turns of the yarns as indicated by the arrows.

5 If a rope made in accordance with my invention be cut across we would find that the following relative arrangement of the yarns in the strand or strands composing the rope:

As shown, the yarns *z* lying more or less on 10 a concentric circle *e* which divides the area of the strand equally, the fibers are straight, that is, have no twist at all, and the fibers of the yarns *y* interior of the said circle *e* will have turns in the same direction as the strand 15 *b* with the number of turns progressively increased towards the center of the strand, and the fibers of the yarns *z* lying exterior of said circle will have turns in the opposite direction with the amount of turns progressively increased towards the circumference 20 of the strand.

Such result is attained by the following assumed relative adjustments of the yarns in the strands in the making of the rope.

25 Let it be assumed that in the making of a rope having a circumference of about six inches, that the initial twist of the yarns was one and one-half turns per foot to the left, and the twist of the strand was two turns 30 per foot to the right, and that the relative lengths of the exterior yarns *z* are approximately two feet for every foot of strand, due to the relatively larger spirals formed by the 35 yarns lying at the exterior of the strand.

Similarly the lengths of the yarns per lineal foot of the strand will be relatively less towards the center of the strand until at the center the yarns *y* are equal in length to the lineal foot of the strand.

40 In other words, for every turn put into the strand there will be a corresponding turn put into the yarns forming the strand; and therefore, since the exterior yarns *z* had initially one and one-half turns per foot to the left 45 and are two feet long, they will have three turns to the left for every foot of strand, and the two turns per foot put in the strand in the opposite direction will reduce the number of turns in the exterior yarns to 1 turn in 50 two feet to the left or one-half turn per foot.

Also, the yarns towards the interior of the strand are progressively shorter so the yarns *z* lying approximately on the circle *e* which are only, approximately, one and one-third 55 feet long per foot of strand, and have initially one and one-half turns per foot of yarns to the left will have two turns for every foot of strand, therefore due to the two turns put in the strand in the opposite direction, the 60 yarns *z* will have had all the turns taken out of them and hence the fibers will be straight.

Similarly, the center yarns *y* being approximately only one foot long, per foot of strand, and having initially one and one-half turns 65 per foot they will have only one and one-half

turns for every foot of strand, and the two turns put in the strand in the opposite direction not only take out the original one and one-half turns to the left, but add one-half turn to the right.

70 Thus the yarns all lie closely together and side by side with no interstices between in which moisture may collect to stiffen and harden the fibers, and since none of the yarns cross one another there is no chafing or cutting, or resistance to individual adjustment when the rope is bent:

75 The latter being due to the fact that the change in twist of the yarns throughout the strand is gradual and that while the yarns lie closely together they are not tightly twisted; but lie as a relatively loose homogeneous mass.

I claim:

1. A rope having a strand comprising a plurality of yarns twisted together, the yarns lying in the center of the strand having individual turns in the same direction as the turns of the strand, and the individual turns of the yarns being less from the center of the strand outward until the yarns lying on a circle located concentric with and between the center and the circumference of the strand are without turns, lying in parallel relation and the turns of the yarns lying exterior of said circle being in the opposite direction and gradually increasing towards the circumference of the strand from the yarns lying on the said circle in parallel relation.

90 2. A rope having a strand comprising a plurality of yarns twisted together, the yarns lying in the center of the strand having a lesser number of individual turns than the turns of the strand, but in the same direction, and the individual turns of the yarns being less from the center of the strand outward until the yarns lying on a circle located concentric with and between the center and the circumference of the strand are without turns, lying in parallel relation, and the turns of the yarns lying exterior of said circle being in the opposite direction and gradually increasing towards the circumference of the strand from the yarns lying on the said circle in parallel relation, and the number of turns of the yarns at the center of the strand and at the circumference being equal, but in the 95 opposite direction.

100 3. A rope having a strand comprising a plurality of yarns twisted together, the yarns lying in the center of the strand having a lesser number of individual turns than the turns of the strand but in the same direction, and the individual turns of the yarns being less from the center of the strand outward until the yarns lying on a circle located concentric with and between the center and the circumference of the strand, and dividing the cross sectional area of the strand 105 110 115 120 125 130

equally are without turns, lying in parallel relation, and the turns of the yarns lying exterior of said circle being in the opposite direction and gradually increasing towards the circumference of the strand from the yarns lying on the said circle in parallel relation, and the number of turns of the yarns at the center of the strand and at the circumference being equal, but in the opposite direction.

10 HENRY S. MEARS.

15

20

25

30

35

40

45

50

55

60

65